

1

3,600,174

**HIGH-CONTRAST PHOTOGRAPHIC ELEMENTS  
AND METHOD FOR PROCESSING SAME**  
Kirby M. Milton, Rochester, N.Y., assignor to  
Eastman Kodak Company, Rochester, N.Y.  
No Drawing. Filed Aug. 18, 1967, Ser. No. 661,531  
Int. Cl. G03c 5/24, 5/26

U.S. Cl. 96—50

14 Claims

## ABSTRACT OF THE DISCLOSURE

High-contrast photographic elements comprising a support coated with a silver halide emulsion wherein the halide comprises at least about 85 mole percent chloride and having a heavy overcoat of a water-permeable colloid. Methods for processing these elements in a continuous transport processing machine wherein the developer contains a carbonyl bisulfite-amine condensation product are also described.

## BACKGROUND OF THE INVENTION

### Field of the invention

This invention relates to photographic materials, their preparation and use. One aspect of the invention relates to a continuous process for processing exposed high-contrast photographic elements in a continuous transport processing machine wherein certain developers must be employed in combination with photographic elements having certain silver halide emulsions and having an overcoating of a specific weight in order to increase effective contrast, eliminate or reduce drag lines, improve dot quality, provide incubation stability, increase speed and improve the shape of its H and D curve. Another aspect of the invention relates to the high-contrast photographic elements themselves.

### Description of the prior art

In the graphic arts field, where it is desired to make photographic line and halftone reproductions, it is customary to employ emulsions having extremely high contrast. In development, the developing areas grow autocatalytically at a very high developing rate to produce an extremely high contrast which is necessary for halftone patterns. Developers for use with extremely high-contrast photographic films are quite different in composition from typical black-and-white film developers. In order to obtain very high contrast and sharp halftone dots, it has been the practice to formulate developers for such films from essentially hydroquinone, an alkali, an alkali metal bromide and a low level of sulfite ion. The low level of sulfite ion partially stabilizes the developer solution for a short period of time and is achieved in all known commercial developers of this type by the use of sodium formaldehyde bisulfite, which acts as a sulfite ion buffer. These developer solutions must be stored in two parts, however, since the sodium formaldehyde bisulfite will dissociate at a high pH to give not only the desired sulfite ion but an equimolar amount of formaldehyde which will react with hydroquinone to destroy its developing power.

In reproducing continuous tone material, it is customary to make a halftone photographic intermediate, usually a film negative, in which the gradations in tone are represented by differing sizes of dots of uniform density. The shape, density and uniformity of the halftone dots are closely correlated to the quality of the resulting picture.

The developer solutions for high-contrast films presently used in continuous transport processing machines also have a number of disadvantages. The photographic

2

quality obtained with a given film is usually inferior to that obtained in careful tray processing. The sensitivity of high-contrast films to developer exhaustion products and variations in local developing agent concentration makes these films vulnerable to directional drag streaks in film halftone areas under conditions of machine processing. These drag streaks occur in areas of high development (50–90% dots) which are adjacent to areas of low development (dot area of 20% or less). The drag streaks are formed by more development occurring because the developer which is "dragged in" from the area of low development contains more developing agent and less exhausting products (primarily bromide ion) than the developer that would normally be in that area. The dots in a high-contrast film are also distorted and exhibit size changes depending on the orientation and direction of travel through the machine processor. This dot distortion is a manifestation of discontinuities or plateaus in the H and D curve of high-contrast films which are processed in continuous transport processing machines. The elimination or reduction of drag streaks and dot distortions would be a considerable advance in the art.

U.S. Pat. 3,058,826 of Meerkamper et al. issued Oct. 16, 1962, discloses the use of heavy gelatin overcoats to reduce haze in photographic elements caused by certain addenda. There is no disclosure in this patent, however, of the high-contrast elements having the specific silver halide emulsions taught herein and having a heavy overcoat of a water-permeable colloid or of processing these elements in a continuous transport processing machine employing only certain developers to provide the improvements taught by the instant invention.

## SUMMARY OF THE INVENTION

In my invention, there are provided high-contrast photographic elements comprising a support coated with a silver halide emulsion having an overcoating comprising a water-permeable colloid coated over the emulsion layer in an amount of at least about 130 milligrams of colloid per square foot, said halide comprising at least about 85 mole percent chloride. I also provide a continuous process for processing such elements, after exposure, in one continuous motion by transporting them into and out of at least one processing solution in the manner shown, for example, by U.S. Pats. 3,025,779 of Russell and Kunz issued Mar. 20, 1962; 3,078,024 of Sardeson issued Feb. 19, 1963; 3,122,086 of Fitch issued Feb. 25, 1964; 3,149,551 of Cramer issued Sept. 22, 1964; 3,156,173 of Meyer issued Nov. 10, 1964; and 3,224,356 of Fleisher and Hixon issued Feb. 21, 1965; and wherein said elements are developed in a liquid developer composition comprising a developing agent and a carbonyl bisulfite-amine condensation product.

## DESCRIPTION OF THE PREFERRED EMBODIMENTS

The developing agents which can be employed in the instant invention can be any of those suitable for the intended purpose. Useful silver halide developing agents, for example, include the dihydroxybenzenes such as hydroquinone; chlorohydroquinone; bromohydroquinone; isopropylhydroquinone; toluhydroquinone; methylhydroquinone; 2,3 - dichlorohydroquinone; 2,5 - dimethylhydroquinone; 2,3 - dibromohydroquinone; 1,4 - dihydroxy - 2-acetophenone - 2,5 - dimethylhydroquinone; 2,5 - diethylhydroquinone; 2,5 - di - p - phenethylhydroquinone; 2,5 - dibenzoylaminohydroquinone; 2,5 - diacetaminohydroquinone; etc. Esters of such compounds, e.g., formates and acetates, can also be employed. These developing agents can be used alone or in any combination and can be employed in any concentration which is effective for development. A suitable concentration for the developing

agent is from about 0.05 to about 0.50 mole per liter of developer composition and is preferably from about 0.10 to about 0.30 mole per liter of developer composition.

The carbonyl bisulfite-amine condensation products which can be used in the developer composition employed in my invention are preferably formaldehyde bisulfite-amine condensation products such as sodium - 2 - hydroxyethylaminomethane sulfonate; sodium - 2 - hydroxypropylaminomethane sulfonate; sodium - 1,1 - dimethyl-2 - hydroxyethylaminomethane sulfonate; sodium - 1,1 - bis - (hydroxymethyl)ethylaminomethane sulfonate; sodium - tris(hydroxymethyl)methylaminomethane sulfonate; sodium - 3 - hydroxypropylaminomethane sulfonate; sodium - bis(2 - hydroxyethyl)aminomethane sulfonate; sodium - N,N - bis[2 - (1 - hydroxy)propyl]aminomethane sulfonate; sodium - N - isopropyl - N - (2 - hydroxyethyl) - aminomethane sulfonate; sodium - N - ethyl - N - (2 - hydroxyethyl) - aminomethane sulfonate; and sodium - N - methyl - N - (2 - hydroxyethyl) - aminomethane sulfonate. The carbonyl bisulfite-amine condensation products can be used alone or in any combination and can be employed in any concentration which is effective to provide a low level of sulfite ion for the developer composition. A suitable concentration for the carbonyl bisulfite-amine condensation product is from about 0.1 to about 1.0 mole per liter of liquid developer composition and is preferably from about 0.25 to about 0.50 mole per liter of liquid developer composition.

The carbonyl bisulfite-amine condensation product can be added to the developer composition as a separate compound or formed in situ. Methods for preparing these compounds are disclosed, for example, in U.S. Pat. No. 2,388,816 of Bean issued Nov. 13, 1945. In this specification and claims, it is meant to include within the definition of carbonyl bisulfite-amine condensation product either the compound itself or the individual components which form the compound in situ.

The high-contrast photographic elements of the instant invention comprise a support coated with a silver halide emulsion layer in which the halide comprises at least about 85 mole percent chloride. Preferably, the halide in said silver halide emulsion comprises at least about 90 mole percent chloride, the balance, if any, being bromide. Such preferred emulsions provide particularly good results in eliminating drag streaks and dot distortions. The halide of said silver halide emulsion can also contain a small amount of iodide, e.g., less than about 5 mole percent, if desired. Silver halide emulsions wherein the halide comprises 100 mole percent chloride have also been found to be quite useful.

The silver halide emulsion layer of the high-contrast photographic elements of the instant invention can contain any of hydrophilic water-permeable binding materials suitable for this purpose. Suitable materials include gelatin, colloidal albumin, polyvinyl compounds, cellulose derivatives, acrylamide polymers, etc. Mixtures of these binding agents can also be used. The binding agents for the emulsion layer of the high-contrast photographic element can also contain dispersed polymerized vinyl compounds. Such compounds are disclosed, for example, in U.S. Pats. 3,142,568 of Nottorf issued July 28, 1964; 3,193,386 of White issued July 6, 1965; 3,062,674 of Houck, Smith and Yudelson issued Nov. 6, 1962; and 3,220,844 of Houck, Smith and Yudelson issued Nov. 30, 1965; and include the water-insoluble polymers of alkyl acrylates and methacrylates, acrylic acid, sulfoalkyl acrylates or methacrylates, interpolymers of alkyl acrylates with acrylic acids, acryloyloxy alkyl sulfonic acids, acetoacetoxy alkyl acrylates such as 2-acetoacetoxyethyl methacrylate and the like. These compounds can also be incorporated into a separate layer of the photographic element. The vinyl polymers are generally employed in concentrations in the range of about 20 to about 80%, most often concentrations at least 50%, by weight, based on the weight of the binding agent. Silver halide emul-

sions wherein the binding agent contains a dispersed polymerized vinyl compound provide particularly good results in eliminating drag streaks and dot distortions.

As indicated above, the high-contrast photographic elements of the instant invention have a heavy overcoat comprising a water-permeable colloid. While any of the hydrophilic water-permeable binding materials listed above for the emulsion layer can be used in the overcoat layer, gelatin has been found to give very good results. If desired, the overcoat layer can also contain dispersed polymerized vinyl compounds as listed above.

The overcoat layer of the high-contrast photographic elements of the instant invention is a very important feature of the invention. This overcoat layer is to be distinguished from a gelatin antiabrasion overcoat layer, known in the art, which is generally coated in such a manner as to give a dry coating weight of not more than 10 milligrams per square decimeter (about 96 milligrams per square foot)—see U.S. Pat. No. 3,058,826 of Meerkamper et al. issued Oct. 16, 1962, column 1, lines 37-41. The overcoat layer of my invention contains at least about 130 to about 460 milligrams of water-permeable colloid based on dry weight per square foot. Higher concentrations can also be employed if desired.

The silver halide emulsion of the high-contrast photographic elements of the instant invention can be coated on a wide variety of supports. Hydrophilic colloid layers can be coated on one or both sides of the support, if desired. Typical supports are cellulose nitrate film, cellulose ester film, polyvinyl acetal film, polystyrene film, poly(ethylene terephthalate) film, and related films or resinous materials, as well as glass, paper, metal and the like. Supports such as paper, which are coated with  $\alpha$ -olefin polymers, particularly polymers of  $\alpha$ -olefins containing two or more carbon atoms, as exemplified by polyethylene, polypropylene, ethylene-butene copolymers and the like can also be employed.

The silver halide emulsions of the high-contrast photographic elements of the instant invention can be sensitized using any of the well-known techniques in emulsion making, for example, by digesting with naturally active gelatin or various sulfur, selenium, tellurium compounds and/or gold compounds. The emulsions can be sensitized with salts of noble metals of Group VIII of the Periodic Table which have an atomic weight greater than 100. The emulsions can also contain addenda which increase speed and/or contrast such as quaternary ammonium salts, polyethylene glycols, thioether sensitizers or combinations thereof.

The silver halide emulsion of the high-contrast photographic elements of the instant invention can conveniently be ortho-sensitized or para-sensitized with spectral sensitizing dyes. For instance, these emulsions can be spectrally sensitized by treating with a solution of a sensitizing dye in an organic solvent. Sensitizing dyes useful in sensitizing such emulsions are described, for example, in U.S. Patents 2,526,632 of Brooker and White issued Oct. 24, 1950, and 2,503,776 of Sprague issued Apr. 11, 1950. Spectral sensitizers which can be used are the cyanines, merocyanines, complex (trinuclear) cyanines, complex (trinuclear) merocyanines, styryls, and hemicyanines.

The silver halide emulsion of the high-contrast photographic elements of the instant invention can also contain conventional addenda such as gelatin plasticizers, coating aids, antifoggants such as the azaindines and hardeners such as aldehyde hardeners, e.g., formaldehyde, mucochloric acid, glutaraldehyde bis(sodium bisulfite), maleic dialdehyde, aziridines, dioxane derivatives and oxypoly-

70 saccharides.

75 Other methods for reducing or eliminating drag streaks and dot distortions in continuous transport processing machines are found in application Ser. No. 661,532 of my co-worker Masset, filed concurrently herewith and entitled "Photographic Developer Composition and Process

of Using Same"; application Ser. No. 661,530 of my co-worker Salesin, filed concurrently herewith and entitled "High-Contrast Photographic Elements and Method for Processing Same"; and my application Ser. No. 661,533 filed concurrently herewith and entitled "Method for Processing High-Contrast Photographic Elements (Case B)."

This invention can be further illustrated by the following examples of preferred embodiments thereof although it will be understood that these examples are included merely for purposes of illustration and are not intended to limit the scope of the invention unless otherwise specifically indicated.

#### EXAMPLE 1

A fine-grain silver chlorobromoiode gelatin emulsion containing 90 mole percent chloride, 9 mole percent bromide and 1 mole percent iodide is chemically sensitized with sulfur and gold compounds and coated on a polyethylene terephthalate support at a coverage of 470 milligrams of silver per square foot and 466 milligrams of gelatin per square foot. A gelatin overcoat is coated over the emulsion layer at 82.5, 165 and 247.5 milligrams of gelatin per square foot. These elements are referred to as A, B and C, respectively.

The coated elements are then exposed, using tungsten illumination, to a step wedge through a magenta contact screen. The elements are then processed using a 90-second development time in a Kodalith Roller Transport 324 Film Processor, of the type shown in U.S. Pat. 3,025,779 of Russell and Kunz issued Mar. 20, 1962, employing the following developer which is disclosed and claimed in my co-worker Masseth's copending application Ser. No. 661,532 filed concurrently herewith and entitled "Photographic Developer Composition and Process of Using Same":

Sodium-bis-(2-hydroxyethyl)-aminomethane sulfonate: 1  
82.0 grams  
Sodium sulfite: 30.0 grams  
Boric acid: 7.5 grams  
Hydroquinone: 22.5 grams  
Potassium bromide: 1.6 grams  
2,2'-iminodiethanol: 39.0 grams  
Water to make: 1 liter  
pH: 9.5

The processed element consists of a pattern of dots, areas commonly referred to as shadow dots and areas known as high-light areas. The quality of reproduction is measured by examining the dot areas and assigning a number ranging from 9 (Excellent) to 1 (Extremely Poor). In the table, H, M and S refer to high-light, middle tone and shadow dots respectively. The following results are obtained:

| Element | Gelatin overcoat (mg.) | Relative speed | Effective contrast <sup>1</sup> | Dot quality |   |   | Drag lines |
|---------|------------------------|----------------|---------------------------------|-------------|---|---|------------|
|         |                        |                |                                 | H           | M | S |            |
| A-----  | 82.5                   | 100            | 1.22                            | 8           | 8 | 7 | Severe.    |
| B-----  | 165                    | 324            | 7.50                            | 9           | 9 | 9 | None.      |
| C-----  | 247.5                  | 100            | 9.80                            | 9           | 9 | 9 | Do.        |

<sup>1</sup> Slope of the straight line between two points which are 0.3 Log E apart of the D vs. Log E curve, where the lower point has a density of 0.1 above fog.

The above results show that increasing the gelatin overcoat increases effective contrast, eliminates drag lines, improves dot quality and increases speed at certain thicknesses.

#### EXAMPLE 2

Coated elements similar to A and C in Example 1 are prepared, exposed and processed as in Example 1 using a 105-second development time. Similar coatings are subjected to natural aging conditions before testing and a third set to 120° F. and 50% relative humidity incuba-

tion for one week before testing. The following results are obtained:

| Element | Gelatin overcoat (mg.) | Relative speed |               |     | 1 week at 120° F./50% relative humidity |
|---------|------------------------|----------------|---------------|-----|-----------------------------------------|
|         |                        | Fresh          | 17 days aging | 115 |                                         |
| A-----  | 82.5                   | 100            | 55            | 41  |                                         |
| C-----  | 247.5                  | 115            | 115           | 115 |                                         |

The above results show that a heavy gelatin overcoat provides incubation stability.

#### EXAMPLE 3

Example 1 is repeated but with half of the gelatin in the overcoat replaced with a dispersed polymerized vinyl compound such as copoly(methyl acrylate-sulfopropyl acrylate). Results similar to those of Example 1 are obtained thus illustrating that synthetic vehicles can be substituted for some of the gelatin in the overcoat with no adverse affects.

#### EXAMPLE 4

Coated elements similar to A and C in Example 1 are prepared, exposed and processed as in Example 1 employing the following developer:

Sodium -  $\beta$  - hydroxyethylaminomethane sulfonate: 322 grams  
Hydroquinone: 90 grams  
Potassium bromide: 6.3 grams  
Water to make: 1 liter  
pH: 16.0<sup>2</sup>

The following results are obtained at a development time of 2 1/4 minutes:

| Element | Gelatin overcoat (mg.) | Effective contrast | Curve shape |     |
|---------|------------------------|--------------------|-------------|-----|
|         |                        |                    | 3.3         | 6.1 |
| A-----  | 82.5                   | 3.3                | Poor.       |     |
| C-----  | 247.5                  | 6.1                | Fair.       |     |

#### EXAMPLE 5

(A) A fine-grain silver chlorobromoiode gelatin emulsion containing 90 mole percent chloride, 9 mole percent bromide and 1 mole percent iodide is chemically sensitized as in Example 1 and coated on a polyethylene terephthalate support at a coverage of 456 milligrams of silver per square foot and 452 milligrams of gelatin per square foot. Gelatin overcoats are then coated over the emulsion layer of portions of the sample at coverages of 83 milligrams per square foot (normal overcoat) and 248 milligrams per square foot (heavy overcoat).

(B) Coated elements similar to (A) are prepared but with 80 mole percent chloride, 19 mole percent bromide and 1 mole percent iodide.

(C) Coated elements similar to (A) are prepared but with 70 mole percent chloride, 29 mole percent bromide and 1 mole percent iodide.

(D) Coated elements similar to (A) are prepared but with 40 mole percent chloride, 59 mole percent bromide and 1 mole percent iodide.

The coated elements are then exposed and processed as in Example 1 employing a 1 1/4-minute development time with the following results:

| Coated Element | Mole percent Cl/Br/I | Gelatin overcoat (mg./ft. <sup>2</sup> ) | Relative speed | Contrast | Dot quality |
|----------------|----------------------|------------------------------------------|----------------|----------|-------------|
| A-----         | 90/9/1               | 83                                       | 100            | 2.67     | 19          |
| A-----         | 90/9/1               | 248                                      | 209            | 10.7     | 8           |
| B-----         | 80/19/1              | 83                                       | 36             | 3.45     | 8           |
| B-----         | 80/19/1              | 248                                      | 91             | 5.8      | 4           |
| C-----         | 70/29/1              | 83                                       | 32             | 4.8      | 7           |
| C-----         | 70/29/1              | 248                                      | 80             | 4.9      | 2           |
| D-----         | 40/59/1              | 83                                       | 16             | 3.10     | 1           |
| D-----         | 40/59/1              | 248                                      | 28             | 2.58     | 1           |

<sup>1</sup> This sample has a very poor curve shape.

<sup>2</sup> pH adjusted with sodium carbonate.

<sup>1</sup> Sodium formaldehyde bisulfite and 2,2'-iminodiethanol can be used to form this compound in situ.

The above results indicate that high-contrast photographic elements wherein the silver halide emulsion is overcoated with a heavy layer of a water-permeable colloid and wherein the halide comprises at least 85 mole percent chloride provides significant increases in relative speed, contrast and dot quality.

Although the invention has been described in considerable detail with particular reference to certain preferred embodiments thereof, variations and modifications can be effected within the spirit and scope of the invention as described hereinbefore and as defined in the appended claims.

I claim:

1. A high-contrast, photographic element comprising a support coated with a silver halide emulsion layer, said halide comprising at least about 85 mole percent chloride, and said element having an overcoating comprising gelatin coated over said emulsion layer in an amount of at least about 130 milligrams per square foot.

2. The photographic element of claim 1 wherein said gelatin overcoating contains from about 130 to about 460 milligrams of gelatin per square foot.

3. The photographic element of claim 1 wherein said halide comprises about 90 mole percent chloride, about 1 mole percent iodide and about 9 mole percent bromide.

4. In a continuous process for processing an exposed, high-contrast, photographic element comprising a support coated with a silver halide emulsion layer wherein said element is processed in one continuous motion by transporting it into and out of at least one processing solution, the improvement comprising:

- (a) developing said element in a liquid developer composition comprising a developing agent and a carbonyl bisulfite-amine condensation product,
- (b) said halide comprising at least about 85 mole percent chloride, and
- (c) said element having an overcoating comprising gelatin coated over said emulsion layer in an amount of at least about 130 milligrams of colloid per square foot.

5. The process of claim 4 wherein said developing agent is a dihydroxybenzene developing agent and said carbonyl bisulfite-amine condensation product is a formaldehyde bisulfite-amine condensation product.

6. The process of claim 5 wherein said dihydroxybenzene developing agent is present in a concentration of from about 0.05 to about 0.50 mole per liter of developer composition and said formaldehyde bisulfite-amine condensation product is present in a concentration of from about 0.10 to about 1.0 mole per liter of developer composition.

7. The process of claim 6 wherein said dihydroxybenzene developing agent is hydroquinone.

8. The process of claim 7 wherein said formaldehyde bisulfite-amine condensation product is sodium bis(2-hydroxyethyl)aminomethane sulfonate.

9. The process of claim 6 wherein said photographic element is transported by rollers.

10. The process of claim 5 wherein said gelatin overcoating contains from about 130 to about 460 milligrams of gelatin per square foot.

11. The process of claim 7 wherein said gelatin overcoating contains from about 130 to about 460 milligrams of gelatin per square foot.

12. The process of claim 5 wherein said overcoating comprises gelatin and a dispersed water-soluble polymer of an alkyl acrylate, methacrylate, sulfoalkyl acrylates and methacrylates or acrylic acid.

13. The process of claim 12 wherein said vinyl compound is a water-insoluble polymer of an alkyl acrylate or alkyl methacrylate.

14. The process of claim 11 wherein said halide comprises about 90 mole percent chloride, about 1 mole percent iodide and about 9 mole percent bromide.

#### References Cited

##### UNITED STATES PATENTS

|           |         |                  |       |        |
|-----------|---------|------------------|-------|--------|
| 3,393,073 | 7/1968  | Reutenaer et al. | ----- | 96—114 |
| 3,443,946 | 5/1969  | Grabhofer et al. | ----- | 96—50  |
| 3,411,911 | 11/1968 | Dykstra          | ----- | 96—87  |
| 2,388,816 | 11/1945 | Bean             | ----- | 95—88  |
| 3,030,209 | 3/1962  | Henn et al.      | ----- | 96—114 |

40 NORMAN G. TORCHIN, Primary Examiner

E. C. KIMLIN, Assistant Examiner

U.S. Cl. X.R.

96—63, 66, 87